

April 17, 1956

P. D. ZEMANY

2,742,585

ELECTRICAL VAPOR DETECTOR

Filed Aug. 22, 1952



Inventor:  
Paul D. Zemany,  
by *Paul A. Frank*  
His Attorney.

1

2,742,585

## ELECTRICAL VAPOR DETECTOR

Paul D. Zemany, Schenectady, N. Y., assignor to General Electric Company, a corporation of New York

Application August 22, 1952, Serial No. 305,883

8 Claims. (Cl. 313—7)

My invention relates to improvements in electrical vapor detectors for detecting certain substances or impurities in gases disclosed in U. S. Patent 2,550,498, issued April 24, 1951, to Chester W. Rice and assigned to the assignee of my present invention.

In the Rice patent, there are disclosed methods and apparatus for detecting substances such as certain gases, vapors, smokes and similar matter in an atmosphere by directing a sample of an atmosphere suspected of containing a concentration of the substances to be detected into an electrical discharge device under conditions which permit the substance to induce positive ion formation at a more positively charged and heated electrode or anode, the positive ions so formed being collected by a negatively charged electrode to produce an indicating current which increases with the concentration of the substance. Devices of this type have been found to be qualitatively selective at atmospheric or greater pressures and in vacua; that is, they respond only to certain types of substances such as the alkali metals or other substances having ionization potentials less than the electron work function of the electrodes, the halogens or compounds of either. For certain substances such as the alkali metals and their compounds the ion formation apparently occurs by ionization of the substance when it comes into contact with the more positively charged and heated electrode. For others such as the halogens and their compounds the substance appears to cause ion formation only in the presence of what might be called sensitizing materials such as the alkali metals and their compounds, and it further appears in this case that the sensitizing materials themselves are actually ionized to afford the desired positive ion current.

While the above-described device has proved to be quite successful for the qualitative detection of certain substances at atmospheric or greater pressures and in vacua, certain improvements are desirable to facilitate its use in vacua for the detection of halogens and their compounds.

In employing the above-referenced and described device for the detection of halogens and their compounds in vacua, particularly at pressures of the order of 1 mm. Hg. or lower, I have found that high background currents of positive ions are obtained as a result of the absorption of the halogens and their compounds by the large bulk of sensitizing material which is utilized. The large bulk of sensitizing material serves as a source of the halogens and their compounds for a considerable length of time following cessation of their admission to the electrical discharge device and the associated vacuum system, whereby high background currents of positive ions result and limit the usefulness of the device. Moreover, I have found that close spacing of the negative and positive electrodes for the purpose of increasing sensitivity and reducing the difference of potential required to collect the positive ions necessitates elaborate and expensive manufacturing procedures for obtaining such close spacings.

The principal object of my invention is to provide an improved electrical vapor detector of the type described

2

wherein high background currents are absent and expensive manufacturing procedures are avoided.

According to one important aspect of my invention which is more particularly described hereinafter, I eliminate high background currents and expensive manufacturing procedures in vapor detectors of the type described by coating the positive heated electrode with a refractory material which serves both as an insulator and as a long-life positive ion emitter or sensitizing material at the 5 temperature of operation of the device. In this manner I am able to construct the positive and negative electrodes without taking special precautions to prevent their 10 contact with each other and am additionally able to avoid the use of a large bulk of sensitizing material within the 15 discharge device of the detector.

In the single figure of the drawing, which is a partly schematic simplified representation of an electrical vapor detector according to my invention, there is shown an electric discharge device which comprises a hermetically sealed envelope 1 adapted to be sealed into a vacuum system (not shown) through a tubular connection 2. Supported within envelope 1 by means of rigid conductive leads 3 and 4 is a filament 5 which is coated over its operative portions with a refractory material that will 20 be more fully described hereinafter. Surrounding filament 5 is a tubular collector electrode 6 of conductive material such as nickel, copper, silver, platinum, etc., which is supported by a rigid conductive lead 7. As shown, the coating on filament 5 can contact electrode 6 25 at several points. Filament 5 is heated by passing current therethrough from a suitable source 8 of alternating or direct current connected across leads 3 and 4. Interconnecting leads 3 and 7 is a series circuit which includes a source of direct voltage 9, a current limiting resistor 10 30 and a direct current microammeter 11. Lead 3 can be connected to ground as illustrated at 12. Electrode 6 must be at a negative potential with respect to filament 5 and therefore, if source 8 is an alternating voltage source, the peak magnitude must be less than the voltage 35 of source 9 by the desired minimum difference of potential between electrode 6 and filament 5.

In the operation of the device of the drawing, the device is evacuated through tubular connection 2, preferably to a pressure of the order of 1 mm. Hg or lower. After 40 evacuation and energization of the device such that filament 5 heats the coating thereon to a temperature ranging from about 700° C. to 1200–1300° C. or somewhat higher, relatively large ion currents are initially collected upon the negatively charged electrode 6 and indicated 45 upon microammeter 11. When this initial current subsides, the device is prepared to indicate the subsequent admission of the vapors of halogens and their compounds to the vacuum system. Such admission of the vapors of 50 halogens and their compounds causes an increase in the positive ion current collected upon the negatively charged electrode 6. One convenient manner of utilization of the 55 device is to go over the surface of the vacuum system with a probe-directed stream of a gaseous halogen compound such as dichlorodifluoromethane, whereby leaks in the 60 system can be detected by the increase in the reading of meter 11.

One of the most important aspects of my invention concerns the selection of material for coating filament 5 over the portion of its surface which is within electrode 6. This coating according to the invention serves as a 65 source of the alkali metal (e. g. sodium, potassium, etc.) ions or alkali metal compound ions which are collected upon electrode 6 and also as an insulator for preventing electronic conduction between filament 5 and electrode 6. 70 When the vapors of halogens and their compounds come into contact with the heated coating, the evaporation of alkali ions from the surface of the coating increases

thereby increasing the reading of meter 11 and indicating the presence of the halogens. I have found that thin refractory coatings, e. g. coatings of a few mils thickness, of specific metal oxides act both as insulators and alkali ion emitters at temperatures ranging from about 700° C. to 1200-1300° C. or higher. Moreover, although the quantity of the material of the refractory coating is relatively small in volume, alkali ion emission can be obtained for as long as several hundred hours.

Materials which can be alternatively employed for the refractory coating of filament 5 according to the invention are the oxides of aluminum (alumina), titanium (titania), beryllium (beryllia), thorium (thoria), magnesium (magnesia), calcium, molybdenum, iron, manganese, silicon, cobalt, nickel, and the rare earths (the rare earths have atomic numbers 57 to 71, inclusive, e. g. europium, cerium, gadolinium, etc.). Even in their most purified available forms, these oxides contain at least a few hundredths of a per cent of alkali impurities which evaporate as alkali ions during operation of the vapor detector to detect halogens. At the high temperatures of the coating during operation of the device, the oxides of these materials apparently possess semi-conductor properties which allow them to serve as insulators for the direct flow of current between filament 5 and electrode 6 but still permit the evaporation of alkali ions in the presence of halogens. While I do not fully understand the reasons for this dual nature of these materials, I realize that, if these materials remained relatively perfect insulators at high temperatures, continued alkali ion emission could not be obtained because the charge left by removal of a few positive ions from the surface of the coating would effectively prevent further evaporation. Therefore, at the above specified temperatures these materials presumably become sufficiently good semi-conductors to allow migration of charge from the surface of the coating to the filament where the charge is neutralized, but at the same time retain sufficient insulating properties to prevent electronic conduction between filament 5 and electrode 6 where the coating contacts electrode 6. For reasons of which I am not aware, the oxides of zirconium and hafnium do not serve as successful alkali ion emitters in the device of the invention. In any event, the process of the evaporation of alkali ions from the above-mentioned materials is fundamentally different from the evaporation of positive ions from the surface of a conductor.

The thickness of the coating upon filament 5 is, as stated heretofore, preferably of the order of a few mils. The thickness should be as small as possible in order to reduce the bulk of absorbent material within the discharge device but still provide adequate alkali ion emission and insulation. The temperature to which the coating is heated preferably is as high as can be utilized without evaporation of the molecules of the selected material itself, i. e. the material must remain thermally stable. For the materials of the invention this temperature ranges from about 700° C. to about 1300° C. The material of filament 5 must, of course, be a conductor capable of withstanding the high temperatures of operation, e. g. tungsten, platinum, etc. The selected material of the coating can be deposited upon the filament in conventional fashion for oxide-coated filaments by spraying or otherwise applying a colloidal suspension of granules of the material upon the filament and thereafter baking to evaporate the liquid carrier. The filament can have convenient forms or shapes other than the twisted configuration illustrated in the figure, providing sufficient passages are provided within electrode 6 to permit exposure of considerable surface of the coating to vapors of halogens or their compounds introduced into the vacuum system. While it is preferable for electrode 6 to be tubular so that a maximum number of alkali ions evaporated from the coating can be collected, semi-tubular or other convenient shapes can be utilized.

A partial list of halogen compounds to which the device

is sensitive is as follows: chloroform ( $\text{CHCl}_3$ ), ferric chloride ( $\text{FeCl}_3$ ), hydrochloric acid ( $\text{HCl}$ ), bromobenzene ( $\text{C}_6\text{H}_5\text{Br}$ ), methyl iodide ( $\text{CH}_3\text{I}$ ), monochlorobenzene ( $\text{C}_6\text{H}_5\text{Cl}$ ), methylene chloride ( $\text{CH}_2\text{Cl}_2$ ), methyl chloride ( $\text{CH}_3\text{Cl}$ ), chlorodifluoro methane ( $\text{CHClF}_2$ ), and trichloroethylene ( $\text{CHClCCl}_2$ ).

As an example for the purpose of illustration only, I have used a direct voltage of 4.5 volts for source 8 and a direct voltage of 15 volts for source 9. With the device 10 of the invention connected to a vacuum system in which the pressure was about  $1 \times 10^{-6}$  mm. Hg, I observed a reading of 1.10 microamperes upon meter 11. On introducing a small pressure of chlorobenzene in the order of  $10^{-7}$  mm. Hg the reading of meter 11 increased to 1.60 microamperes.

While I have shown and described particular embodiments of my invention, it will be obvious to those skilled in the art that various changes and modifications can be made without departing from the invention and I, therefore, aim in the appended claims to cover all such changes and modifications as fall within the true spirit and scope of the invention.

What I claim as new and desire to secure by Letters Patent of the United States:

- 25 1. In apparatus for selectively detecting halogen vapors and their compounds, an electrical discharge device comprising an evacuable envelope having a conduit opening thereinto for the introduction of vapors to be detected, positive ion generating means supported within said envelope and consisting of a filament coated with a coating a few mils thick of a refractory material selected from the group consisting of the oxides of aluminum, titanium, beryllium, thorium, magnesium, calcium, molybdenum, iron, manganese, silicon, cobalt, nickel and the rare earths, and which contains at least several hundredths percent of an alkali, said coated filament being the only positive ion emitter present within said envelope, and a positive ion collector electrode supported within said envelope closely adjacent to said coated filament.
- 30 2. In a vapor detector wherein alkali ions are selectively formed and collected in the presence of vapors of halogens and their compounds, an electrical discharge device comprising an evacuable envelope having a conduit opening thereinto for the introduction of vapors to be detected, positive ion generating means supported within said envelope and consisting of a filament coated with a coating a few mils of thick of a refractory material which is thermally stable at temperatures between 700° C. and 1300° C. and which contains at least several hundredths percent of an alkali, said coated filament being the only positive ion emitter present within said envelope and having both the property of an alkali ion emitter in the presence of vapors of halogens and their compounds and the property of an insulator for electronic conduction at temperatures between 700° C. and 1300° C., and a cylindrical positive ion collector electrode supported within said envelope closely surrounding said coated filament.
- 35 3. In a vapor detector wherein alkali ions are selectively formed and collected in the presence of vapors of halogens and their compounds an electrical discharge device comprising an evacuable envelope having a conduit opening thereinto for the introduction of vapors to be detected, positive ion generating means supported within said envelope and consisting of a filament coated with a coating a few mils thick of a refractory material selected from the group consisting of the oxides of aluminum, titanium, beryllium, thorium, magnesium, calcium, molybdenum, iron, manganese, silicon, cobalt, nickel and the rare earths, and containing at least several hundredths percent of an alkali, said coated filament being the only positive ion emitter present within said envelope and having both the property of an alkali ion emitter in the presence of vapors of halogens and their compounds and the property of an insulator for electronic conduction at temperatures between 700° C. and 1300° C., and a cylindrical positive ion collector electrode supported within said envelope closely surrounding said coated filament.
- 40 4. In a vapor detector wherein alkali ions are selectively formed and collected in the presence of vapors of halogens and their compounds an electrical discharge device comprising an evacuable envelope having a conduit opening thereinto for the introduction of vapors to be detected, positive ion generating means supported within said envelope and consisting of a filament coated with a coating a few mils thick of a refractory material selected from the group consisting of the oxides of aluminum, titanium, beryllium, thorium, magnesium, calcium, molybdenum, iron, manganese, silicon, cobalt, nickel and the rare earths, and containing at least several hundredths percent of an alkali, said coated filament being the only positive ion emitter present within said envelope and having both the property of an alkali ion emitter in the presence of vapors of halogens and their compounds and the property of an insulator for electronic conduction at temperatures between 700° C. and 1300° C., and a cylindrical positive ion collector electrode supported within said envelope closely surrounding said coated filament.
- 45 5. In a vapor detector wherein alkali ions are selectively formed and collected in the presence of vapors of halogens and their compounds an electrical discharge device comprising an evacuable envelope having a conduit opening thereinto for the introduction of vapors to be detected, positive ion generating means supported within said envelope and consisting of a filament coated with a coating a few mils thick of a refractory material selected from the group consisting of the oxides of aluminum, titanium, beryllium, thorium, magnesium, calcium, molybdenum, iron, manganese, silicon, cobalt, nickel and the rare earths, and containing at least several hundredths percent of an alkali, said coated filament being the only positive ion emitter present within said envelope and having both the property of an alkali ion emitter in the presence of vapors of halogens and their compounds and the property of an insulator for electronic conduction at temperatures between 700° C. and 1300° C., and a cylindrical positive ion collector electrode supported within said envelope closely surrounding said coated filament.
- 50 6. In a vapor detector wherein alkali ions are selectively formed and collected in the presence of vapors of halogens and their compounds an electrical discharge device comprising an evacuable envelope having a conduit opening thereinto for the introduction of vapors to be detected, positive ion generating means supported within said envelope and consisting of a filament coated with a coating a few mils thick of a refractory material selected from the group consisting of the oxides of aluminum, titanium, beryllium, thorium, magnesium, calcium, molybdenum, iron, manganese, silicon, cobalt, nickel and the rare earths, and containing at least several hundredths percent of an alkali, said coated filament being the only positive ion emitter present within said envelope and having both the property of an alkali ion emitter in the presence of vapors of halogens and their compounds and the property of an insulator for electronic conduction at temperatures between 700° C. and 1300° C., and a cylindrical positive ion collector electrode supported within said envelope closely surrounding said coated filament.
- 55 7. In a vapor detector wherein alkali ions are selectively formed and collected in the presence of vapors of halogens and their compounds an electrical discharge device comprising an evacuable envelope having a conduit opening thereinto for the introduction of vapors to be detected, positive ion generating means supported within said envelope and consisting of a filament coated with a coating a few mils thick of a refractory material selected from the group consisting of the oxides of aluminum, titanium, beryllium, thorium, magnesium, calcium, molybdenum, iron, manganese, silicon, cobalt, nickel and the rare earths, and containing at least several hundredths percent of an alkali, said coated filament being the only positive ion emitter present within said envelope and having both the property of an alkali ion emitter in the presence of vapors of halogens and their compounds and the property of an insulator for electronic conduction at temperatures between 700° C. and 1300° C., and a cylindrical positive ion collector electrode supported within said envelope closely surrounding said coated filament.
- 60 8. In a vapor detector wherein alkali ions are selectively formed and collected in the presence of vapors of halogens and their compounds an electrical discharge device comprising an evacuable envelope having a conduit opening thereinto for the introduction of vapors to be detected, positive ion generating means supported within said envelope and consisting of a filament coated with a coating a few mils thick of a refractory material selected from the group consisting of the oxides of aluminum, titanium, beryllium, thorium, magnesium, calcium, molybdenum, iron, manganese, silicon, cobalt, nickel and the rare earths, and containing at least several hundredths percent of an alkali, said coated filament being the only positive ion emitter present within said envelope and having both the property of an alkali ion emitter in the presence of vapors of halogens and their compounds and the property of an insulator for electronic conduction at temperatures between 700° C. and 1300° C., and a cylindrical positive ion collector electrode supported within said envelope closely surrounding said coated filament.
- 65 9. In a vapor detector wherein alkali ions are selectively formed and collected in the presence of vapors of halogens and their compounds an electrical discharge device comprising an evacuable envelope having a conduit opening thereinto for the introduction of vapors to be detected, positive ion generating means supported within said envelope and consisting of a filament coated with a coating a few mils thick of a refractory material selected from the group consisting of the oxides of aluminum, titanium, beryllium, thorium, magnesium, calcium, molybdenum, iron, manganese, silicon, cobalt, nickel and the rare earths, and containing at least several hundredths percent of an alkali, said coated filament being the only positive ion emitter present within said envelope and having both the property of an alkali ion emitter in the presence of vapors of halogens and their compounds and the property of an insulator for electronic conduction at temperatures between 700° C. and 1300° C., and a cylindrical positive ion collector electrode supported within said envelope closely surrounding said coated filament.
- 70 10. In a vapor detector wherein alkali ions are selectively formed and collected in the presence of vapors of halogens and their compounds an electrical discharge device comprising an evacuable envelope having a conduit opening thereinto for the introduction of vapors to be detected, positive ion generating means supported within said envelope and consisting of a filament coated with a coating a few mils thick of a refractory material selected from the group consisting of the oxides of aluminum, titanium, beryllium, thorium, magnesium, calcium, molybdenum, iron, manganese, silicon, cobalt, nickel and the rare earths, and containing at least several hundredths percent of an alkali, said coated filament being the only positive ion emitter present within said envelope and having both the property of an alkali ion emitter in the presence of vapors of halogens and their compounds and the property of an insulator for electronic conduction at temperatures between 700° C. and 1300° C., and a cylindrical positive ion collector electrode supported within said envelope closely surrounding said coated filament.

tive ion collector electrode supported within said envelope closely adjacent to said coated filament.

4. The device of claim 3 in which the refractory coating upon the filament is alumina.

5. The device of claim 3 in which the refractory coating upon the filament is titania.

6. The device of claim 3 in which the refractory coating upon the filament is beryllia.

7. The device of claim 3 in which the refractory coating upon the filament is thoria.

8. The device of claim 3 in which the refractory coating upon the filament is magnesia.

References Cited in the file of this patent

UNITED STATES PATENTS

|           |           |               |
|-----------|-----------|---------------|
| 2,164,913 | Goodchild | July 4, 1939  |
| 2,393,650 | Metcalf   | Jan. 29, 1946 |
| 2,550,498 | Rice      | Apr. 24, 1951 |